

1

2,927,892

## OIL DISPERSIONS OF CALCIUM ACETATE HYDRATES

Arnold J. Morway, Clark, N.J., assignor to Esso Research and Engineering Company, a corporation of Delaware

No Drawing. Application August 6, 1957  
Serial No. 676,475

8 Claims. (Cl. 252—39)

This invention relates to lubricating oil compositions having good load-carrying ability and extreme pressure properties. Particularly, it relates to lubricating oil compositions containing calcium acetate hydrates.

While anhydrous calcium acetate will impart load-carrying ability and improved anti-wear properties to lubricating oil compositions, it will not form stable dispersions in lubricating oil without the aid of other agents such as: emulsifiers (for oil-water dispersions); grease thickeners, e.g. metal salts of  $C_7$  to  $C_{30}$  fatty acids or other suspending aids. However, the emulsion type dispersions have the disadvantages of increased corrosion due to the water and the danger of the emulsion breaking or freezing. The presence of fatty acid salts, or other grease thickener or suspending aids are at times undesirable for certain applications due to side reactions or the formation of residues. It has now been found that excellent dry (i.e. no free water) lubricating compositions containing as the sole salt component either calcium acetate monohydrate, i.e.  $Ca(CH_3COO)_2 \cdot H_2O$ , calcium acetate dihydrate, i.e.,  $Ca(CH_3COO)_2 \cdot 2H_2O$ , or mixtures thereof, will form stable dispersions without the aid of other suspending agents. Also, these hydrates have even better anti-wear and load-carrying ability than the anhydrous calcium acetate. Lubricants of this type are suitable for use in internal combustion engines, textile mill lubricants, and because of their acid neutralizing ability are particularly useful for lubricating the upper cylinders of marine diesel engines operating on acid-forming fuel such as high-sulfur fuel oils, etc.

The compositions of the invention will, therefore, comprise a major proportion of a lubricating oil and about 2 to 40, e.g., 5 to 30 weight percent, based on the weight of the total composition, of either the mono- or dihydrate of calcium acetate, or mixtures thereof.

The lubricating oil used in the compositions of the invention may be either mineral lubricating oil or a synthetic lubricating oil. Synthetic lubricating oils which may be used include esters of dibasic acids (e.g., di-2-ethyl hexyl sebacate), esters of glycols (e.g.  $C_{13}$  Oxo acid diester of tetraethylene glycol), complex esters (e.g. the complex ester formed by reacting one mole of sebacic acid with two moles of tetraethylene glycol and two moles of 2-ethyl-hexanoic acid), halocarbon oils, alkyl silicates, sulfite esters, mercaptals, formals, polyglycol type synthetic oils, etc., or mixtures of any of the above in any proportions.

Other additives may also be added to the lubricating composition in amounts of about 0.1 to 10.0 weight percent or more, for example: oxidation inhibitors such as phenyl alpha naphthylamine; corrosion inhibitors, such

2

as sorbitan monooleate; dyes; viscosity index improvers, detergents and the like.

The calcium acetate hydrates may be preformed and then added directly to the lubricating oil in the desired proportions with stirring. Preferably, because less expensive and easier to suspend, the hydrates are formed in situ in the lubricating oil as follows: A slurry is formed of the oil and a calcium base, such as calcium hydroxide, calcium oxide, calcium carbonate, etc. When the calcium oxide or carbonate is used, a small amount of water may be added in order to furnish the water of hydration. The acetic acid is then added slowly (to prevent overheating) to the slurry while stirring. If the dihydrate is desired, then the temperature of the reaction mixture should not be allowed to exceed about 180°—200° F., as above this temperature the dihydrate tends to lose one mole of the water of hydration and is converted into the monohydrate. If the monohydrate is desired, then the reaction mixture is heated above about 180°—200° F. to form the monohydrate. This monohydrate in turn is relatively stable up to about 300° F. After formation of the calcium acetate hydrate, other additives may then be added to the composition, after which it is cooled. The hydrates may be formed in the lubricating oil in any proportion, however, for plant operation, it is more economical to form a hydrate concentrate, i.e., about 30 to 60 weight percent of the hydrate in the oil, and then to cut the concentrate back by blending with additional lubricating oil to form the final composition. Although not essential, it is also desirable to homogenize either the concentrate or the final cut back composition or both, by means of a Charlotte mill, a Manton-Gaulin homogenizer, a Morehouse mill, etc. By thus homogenizing a more uniform product is obtained with freedom from lumps, undispersed lime, etc.

Both the mono- and dihydrate are useful in the lubricating oil compositions. However, while excellent stable dispersions are formed from the dihydrate, such dispersions tend to be more viscous than dispersions formed with either the monohydrate or anhydrous calcium acetate per se, and when used in relatively large concentrations, e.g., 20 to 40 weight percent, it tends to form solid greases at elevated temperatures. However, this is an advantage when non-flowable lubricants are desired. The monohydrate, on the other hand, forms excellent stable dispersions which show little tendency to solidify upon increasing temperatures, and are particularly desirable for use in equipment normally handling fluid lubricants at elevated temperatures. The anhydrous form of the calcium acetate, while readily dispersed in the lubricating oil, during storage tends to separate from the lubricant and for this reason will not form satisfactory lubricants, particularly when used in low viscosity oils.

The invention will be further understood by the following examples.

## EXAMPLE IA

A base material was prepared as follows: 58.0 weight percent of a mineral lubricating oil (100 SUS at 100° F.) which was a Mid-Continent phenol-extracted type mineral oil distillate and 17.0 weight percent of hydrated lime were added to a kettle and mixed to form a smooth intimate slurry. Then, without external heating, 25.0 weight percent of glacial acetic acid was gradually added taking care not to allow the temperature to rise above

200° F. After all the acetic acid was added, the mixture was allowed to cool to 150° F. where it was stirred for one-half hour while maintaining this temperature by external heating in order to ensure completion of the reaction. At the end of this time the heat was turned off and the reaction mixture was homogenized by passing it through a Gaulin homogenizer operating at 6,000 p.s.i. shear.

#### EXAMPLE IB

25 weight percent of the product of Example IA was diluted with 80 weight percent of additional mineral oil (same oil as used in IA) by simple mixing without heating. This new blend was twice passed through a Gaulin homogenizer operating at 6,000 p.s.i. shear.

#### EXAMPLE IIA

A base material was prepared using the same formulation and method of preparation of Example IA except

10

15

|                                                | Compositions of Calcium Acetate Dispersions (Weight Percent) |      |      |      |      |      |       |
|------------------------------------------------|--------------------------------------------------------------|------|------|------|------|------|-------|
|                                                | IA                                                           | IB   | IIA  | IIB  | IIIA | IIIB | IV    |
| Acetic acid (glacial)                          | 25.0                                                         | 5.0  | 25.0 | 5.0  | 25.0 | 5.0  | 4.50  |
| Hydrated lime                                  | 17.0                                                         | 3.4  | 17.0 | 3.4  | 17.0 | 3.4  | 3.06  |
| Mineral oil (100 SUS at 100° F.)               | 58.0                                                         | 91.0 | 58.0 | 91.0 | 58.0 | 91.0 | —     |
| Mineral oil (80 SUS at 210° F.)                | —                                                            | —    | —    | —    | —    | —    | 51.81 |
| Mineral oil (55 SUS at 210° F.)                | —                                                            | —    | —    | —    | —    | —    | 40.63 |
| Max. temp. manufac-<br>ture, ° F.              | 200                                                          | 200  | 300  | 300  | 350  | 350  | 300   |
| Form of calcium acetate<br>(X-ray diffraction) | (1)                                                          | (1)  | (2)  | (2)  | (3)  | (3)  | (3)   |

1 Dihydrate.

2 Monohydrate.

3 Anhydrous.

Table II

|                                                                          | Properties of Calcium Acetate Dispersions |                         |                              |                         |                         |                         |                         |
|--------------------------------------------------------------------------|-------------------------------------------|-------------------------|------------------------------|-------------------------|-------------------------|-------------------------|-------------------------|
|                                                                          | IA                                        | IB                      | IIA                          | IIB                     | IIIA                    | IIIB                    | IV <sup>1</sup>         |
| Appearance                                                               | Excellent smooth grease.                  | Excellent smooth fluid. | Excellent smooth semi-fluid. | Excellent smooth fluid. | Similar to Example IIA. | Excellent smooth fluid. | Excellent smooth fluid. |
| Viscosity, SUS:                                                          |                                           |                         |                              |                         |                         |                         |                         |
| 100° F.                                                                  | 186.7                                     | —                       | —                            | 150.9                   | —                       | 150.5                   | 84.4                    |
| 210° F.                                                                  | Gels                                      | —                       | —                            | 64.4                    | —                       | 63.7                    | 80.2                    |
| Stability:                                                               |                                           |                         |                              |                         |                         |                         |                         |
| 10 days at 80° F.                                                        | Excellent                                 | —                       | —                            | Excellent               | —                       | Poor <sup>2</sup>       | —                       |
| 20 days at 80° F.                                                        | —                                         | —                       | —                            | —                       | —                       | —                       | Excellent               |
| Centrifuge test: 30 minutes, 1,500 r.p.m., precipitation, weight percent | 0.5                                       | —                       | —                            | 1.0                     | —                       | 5.0                     | —                       |
| 4-ball wear spot test: (1,800 r.p.m.—10 kg.—1 hour—75° C.) mm. dia. scar | 0.43                                      | —                       | —                            | 0.39                    | —                       | 0.52                    | 0.22                    |
| Almen test weight carried                                                | 14                                        | —                       | —                            | 14                      | —                       | 13                      | 14                      |

<sup>1</sup> The product of Example IV had a V.I. of 94, a sulfated ash content of 5.57 wt. percent, and in a 120 hour Caterpillar engine test showed excellent wear reduction of the rings and good cleanliness.

<sup>2</sup> Oil separated from the lubricant.

that the dispersion of the hydrated calcium acetate formed in situ was heated to 300° F. for one-half hour. It was then passed twice through a Morehouse mill set at 0.003" clearance.

#### EXAMPLE IIB

20 weight percent of the product of Example IIA was added to 80 weight percent of mineral oil (same as in IA). This diluted product was passed twice through a Gaulin homogenizer operating at 6,000 p.s.i.

#### EXAMPLE IIIA

The formulation and method of preparation followed in Examples IA and IIA was repeated except that the base material was heated to a temperature of 350° F. for 2 hours in order to completely dehydrate the mixture and to form the anhydrous calcium acetate. This base material was then passed through a Morehouse mill twice.

#### EXAMPLE IIIB

The base product formed in Example IIIA was diluted in the same manner as Example IB.

#### EXAMPLE IV

A base grease containing the monohydrate was formed according to the manner of Example IIA except that a heavier mineral lubricating oil having a viscosity of 80 SUS at 210° F. was used. 18.00 weight percent of this base material was then diluted with 40.63 weight percent of mineral lubricating oil having a viscosity of 55 SUS at 210° F. and 41.37 weight percent of a mineral lubricating oil having a viscosity of 80 SUS at 210° F. The blend was then passed through a Gaulin homogenizer operating at 6,000 p.s.i.

The compositions and physical properties of the above lubricants are listed in the following tables.

40 As seen from the above table, both the calcium monohydrate and dihydrates were superior to the anhydrous calcium acetate in regard to wear and load-carrying ability. Furthermore, these hydrates formed very stable dispersions and gave a much smaller degree of precipitation during the centrifuge test as compared to the anhydrous form.

45 By use of the dihydrate in relatively large proportions, greases may be formed, while the larger proportions of the monohydrate permit the formation of semi-fluid materials. Smaller proportions of either hydrate result in the formation of lubricating fluids. Thus, fluids, semi-fluids and greases may be produced by the method of the invention.

50 What is claimed is:

1. A dry lubricating composition comprising a major proportion of lubricating oil and as a sole salt component about 2 to 40 wt. % calcium acetate hydrate selected from the group consisting of calcium acetate monohydrate, calcium acetate dihydrate and mixtures thereof.
2. A composition according to claim 1, containing 5 to 40 weight percent of said hydrate.
3. A composition according to claim 1, wherein said hydrate is calcium acetate monohydrate.
4. A composition according to claim 1, wherein said hydrate is calcium acetate dihydrate.
5. A composition according to claim 1, wherein said hydrate is formed in situ by the neutralization of acetic acid with a calcium base.
6. A process for preparing a lubricating oil dispersion containing as the sole salt component a calcium acetate dihydrate which comprises neutralizing acetic acid with a calcium base in the presence of water and oil while maintaining the temperature of the reaction below about 200° F.
7. A process for preparing a lubricating oil dispersion containing as the sole salt component a calcium acetate monohydrate which comprises preparing the cal-

clum acetate dihydrate according to the method of claim 6, followed by heating above about 200° F. until said monohydrate is formed.

8. A composition according to claim 1, wherein said lubricating oil is mineral oil.

|             |                    |                |
|-------------|--------------------|----------------|
| 2,384,551   | Jehle              | Sept. 11, 1945 |
| 2,607,735   | Sproule            | Aug. 19, 1952  |
| 2,671,758   | Vinograd           | Mar. 9, 1954   |
| 2,744,870   | Stillebroer et al. | May 8, 1956    |
| 5 2,863,847 | Morway             | Dec. 9, 1958   |

## References Cited in the file of this patent

## UNITED STATES PATENTS

|           |          |              |    |
|-----------|----------|--------------|----|
| 2,079,051 | Sullivan | May 4, 1937  | 10 |
| 2,274,676 | Earle    | Mar. 3, 1942 |    |

## OTHER REFERENCES

Kolloid, Z. Article by P.C.L. Thorn et al., vol. 48, 113-125 (1929), Trans. Faraday Soc., vol. 29, pp. 1101-1107 (1939), Research (London), vol. 2, p. 243 (1949).